

## UNITED STATES PATENT OFFICE.

WILLIAM FOX, OF DETROIT, MICHIGAN.

## PROCESS OF PRODUCING DECORATIVE EFFECTS ON GLASS.

No Drawing.

Application filed June 13, 1924. Serial No. 719,743.

*To all whom it may concern:*

Be it known that I, WILLIAM FOX, a citizen of the United States, residing at Detroit, in the county of Wayne and State of Michigan, have invented a new and useful Improvement in Processes of Producing Decorative Effects on Glass, of which the following is a specification.

The object of the invention is to supply an improved process by which decorative effects on glass may be obtained.

I am, of course, aware that at the present time decorative effects are obtained on glass. It has however been the custom to first prepare the glass with a special solution and then to apply special coloring, or else to apply the coloring and then either burn it, or dissipate it with a solution in order to produce the desired effect.

In the present invention I apply the coloring matter to the reverse side of dry clean glass and effect the blending by the application of air from varying angles. Thus one of the objects of my invention is to supply a simplified process by which artistic effects can be obtained.

With this and other objects in view my invention is hereinafter more fully described and claimed:

I first obtain ordinary oil paints of varying shades, such as red, white, yellow and blue, each of which should be thoroughly mixed and if there is any sediment I prefer to strain the paint. I then take a dry clean piece of glass, onto the reverse side of which I apply my paint. For this purpose I procure a small pointed piece of wood, camel hair brush or the like. This I dip into one of the colors and deposit a drop on the reverse surface of the glass. I then drop another drop of another color onto the first drop, or close beside it, and perhaps a third drop onto the two previous drops or close beside them. I then project air from varying angles, preferably through a flexible tube, towards the colors so as to cause them to intermingle and blend. When the colors have been sufficiently dissipated I apply another drop of any desired color which I blend with those already applied as previously described. I usually commence working at one edge or corner of the glass so that I may continue to work from the colored portion without possibility of part of it having dried before the adjoining portion is colored.

Broadly speaking I prefer to superimpose my colors rather than place them on an adjoining portion of the surface yet uncolored for in this way I find that better blending can be effected; and whereas, throughout my description I have used the work color I find that a judicious application of white paint with the colors will add to the effect.

When the whole of the surface of the glass has been colored it will present an indistinguishable mass of color on the reverse side of the glass to which the paints have been applied. But when turned over and looked at through the glass, not only will there be a great number of varying colors, and shades of color, far in excess of the number of different colored paints applied, but it will be noted that the application of air from varying angles has produced an agatelike or mottling effect as well as blending the colors.

Regarding the application of the air I prefer to use warm moist air at a slight pressure of say one ounce, and I find that very good results may be obtained by blowing with the mouth. While I can accomplish my object by using cool dry air supplied by bellows or the like, the results obtained are inferior. This is attributable to the fact that the warmth and moisture affect the paints and cause better and more thorough blending. The agatelike and mottling effects are of course obtained by the application of the air from constantly varying angles.

When the coloring has been completed over the whole surface, I apply varnish or other adhesive material and therewith secure a protective covering of paper, canvas or other protective material to the painted surface of the glass, for it will be remembered that the paint has been applied to the reverse side.

Moreover, instead of using ordinary oil paints as hereinbefore referred to, I may employ transparent aniline paints if I so wish for the decoration of electric light bowls and other articles.

While in the foregoing description I have described the preferred manner in which my process is performed it is understood however that I may vary my process provided the said variations fall within the scope of what I claim.

Having thus described my invention what I desire to secure by Letters Patent is:

1. A process of producing decorative effects on glass comprising applying drops of paint of various colors on the reverse side of dry clean glass and applying air thereto from varying angles.
2. A process of producing decorative effects on glass comprising applying drops of paint of various colors on the reverse side of dry clean glass and blowing warm moist

air on said paint from constantly varying 10 angles.

In testimony whereof I affix my signature in the presence of two witnesses at Majestic Building, Detroit, Michigan.

WILLIAM FOX.

Witnesses:

MAURICE G. VINCE,  
GERALD S. BALDWIN.